

## UNITED STATES PATENT OFFICE

GARDNER R. ALDEN, OF FRAMINGHAM, AND THOMAS NELSON, OF BOSTON, MASSACHUSETTS, ASSIGNORS TO DENNISON MANUFACTURING COMPANY, OF FRAMINGHAM, MASSACHUSETTS, A CORPORATION OF MASSACHUSETTS

## METHOD OF MAKING NONBLEEDING CREPE PAPER

No Drawing.

Application filed June 15, 1929. Serial No. 371,295.

This invention relates to a method of making non-bleeding crepe paper, by dyeing and fixing in a single operation, and to the creping solutions employed therein.

5 In the prior art it has been proposed (see copending applications of one of us, Serial Nos. 140,040 and 147,959 filed October 7, 1926 and November 1926 respectively), to make crepe paper by the several steps of dyeing the 10 paper, rendering the dyed paper fast by treatment with a fixing reagent or mordant, and creping the paper—the steps being carried out in any desired order of sequence. Such procedures are characterized in general by including three separate stages of treatment, 15 namely, dyeing, fixing and creping.

It is an object of this invention to simplify the procedure of treating such products and more especially to effect the dyeing and fixing in a single step. Other objects will appear from the following disclosure.

By the present invention, it is found that the dyeing and fixing of the paper (up to a certain depth of color) may be advantageously effected in a single operation by employing a creping bath which contains both the required dye and a suitable reagent or mordant, and a protective colloid. The creping bath, for example, may include water as the solvent, 30 a dye (e. g., a basic dye), a protective colloid for the same, which is preferably sufficiently adhesive to serve as a creping medium, (such as hide glue) and a fixing reagent or mordant which may be of the usual type.

35 The fixing agent used will be appropriate to the dye or dyes used, and may consist of a usual mordant or a small amount of a direct dye in some cases. From this, it will be clear that when a solution containing simply a direct dye and a protective colloid may be used as the fixing agent the direct dye should be of such nature and concentration as to be held firmly by the cellulose.

The protective colloid may consist of gum arabic, colloidal castor oil, olive oil, sulphonated oils, ammonium stearate or tri-ethanolamine-oleate, etc., and may also include positively adhesive materials such as glue.

45 Since it is desirable that the dye shall not be in excess of that amount which may be ef-

fectively protected by the colloid from precipitating with the fixing agent, and since the amount of protective colloid used is limited to such amounts as will be free flowing and will not interfere with the creping operation,—the concentration of dye is ordinarily limited to somewhat dilute solutions,—e. g. approximately 1.0% to 0.5% or less.

Typical creping solutions, prepared in accordance with this invention may be composed as follows:

|     |                                                 |            |     |
|-----|-------------------------------------------------|------------|-----|
| I   | Rhodamine 6 GDN                                 | 3.75 oz.   |     |
|     | Pheno fast yellow                               | 5.12 oz.   |     |
|     | Solution of hide glue (1.75<br>lbs. per gallon) | 2 gallons  | 65  |
|     | Calco mordant C (pure)                          | 8 oz.      |     |
|     | Water                                           | 60 gallons | 60  |
| II  | Rhodamine 6 GDN                                 | 4 oz.      |     |
|     | Pheno fast yellow                               | 4 oz.      | 70  |
|     | Solution of hide glue (1.75<br>lbs. per gallon) | 2 gallons  |     |
|     | Tannic acid                                     | 1 lb.      |     |
|     | Water                                           | 60 gallons | 75  |
| III | Auramine O                                      | 2.34 oz.   |     |
|     | Brilliant green crystals                        | 3.0 oz.    |     |
|     | Solution of hide glue (1.75<br>lbs. per gallon) | 2 gallons  |     |
|     | Calco mordant C (pure)                          | 11 oz.     | 80  |
|     | Water                                           | 60 gallons |     |
| IV  | Brilliant green crystals                        | 3 oz.      |     |
|     | Auramine O                                      | 3.34 oz.   |     |
|     | Solution of hide glue (1.75<br>lbs. per gallon) | 2 gallons  | 85  |
|     | Katanol W                                       | 1 lb.      |     |
|     | Water                                           | 60 gallons |     |
| V   | Methylene blue                                  | 12.13 oz.  |     |
|     | Victoria green crystals                         | 4.04 oz.   | 90  |
|     | Solution of hide glue (2<br>lbs. per gallon)    | 3 gallons  |     |
|     | Calco mordant C (pure)                          | 20 oz.     |     |
|     | Water                                           | 60 gallons |     |
| VI  | Direct dye mordant                              |            | 95  |
|     | Victoria green crystals                         | 1.60 oz.   |     |
|     | Niagara sky blue 6 B                            | 1.40 oz.   |     |
|     | Solution of hide glue (1.75<br>lbs. per gallon) | 1 gallon   |     |
|     | Water                                           | 60 gallons | 100 |

In the preparation of the creping solution, it is desirable that the protective colloid shall effectively prevent preliminary action of the fixing agent upon the dye. This is accomplished by first dissolving the dye in water, adding the colloidal solution of glue thereto, and finally adding the fixing agent.

For example, in a preferred procedure of the application of the invention, the basic dye stuff may be dissolved in approximately one-half of the ultimate quantity of water which is to be used. The adhesive solution is then added and the two solutions thoroughly mixed by agitation or stirring. The fixing agent or mordant (preferably free from loading or standardizing materials) is then dissolved in a like amount of water and poured into the mixture gradually, with continuous stirring. If a direct dye is to be used as the fixing agent or as a supplementary fixing agent, it is dissolved and added to the mixture last.

The solution as thus prepared is poured into the usual creping pan, and the tissue dyed and creped in the customary manner.

The solution penetrates and dyes the paper and at the same time provides sufficient adhesiveness to the creping roll to effect a well creped sheet. Upon drying, the colored and creped sheet is "non-bleeding" and the product has a lustrous finish which may be attributed to the adhesion of the same to the smooth and heated creping roll before creping which imparts a polished surface thereto.

The present invention thus provides a non-bleeding crepe paper, which is especially desirable for such purposes as table napkins, table covers, etc. At the same time it avoids the necessity of treating with two or three solutions (e. g. dyeing solution, fixing solution and creping solution) and of adjusting the relative amount of each which is required for a given piece of coloring work. It likewise reduces the amount of dyeing and handling equipment required and decreases the length of the sheet of paper which must be conveyed through the creping apparatus in a wet condition.

We claim:

1. A method of making non-bleeding crepe paper, comprising the steps of treating a sheet of tissue paper with a creping bath characterized by containing a dye, an adhesive protective colloid, and a fixing agent or mordant, and subjecting the treated sheet to the creping operation.

2. A method of making non-bleeding paper, comprising the step of treating a sheet of tissue paper with a bath characterized by containing a dye, a protective colloid, and a fixing agent for said dye.

3. A method of making non-bleeding paper, comprising the step of treating a sheet of tissue paper with a bath characterized by containing a dye, a protective colloid, and a

fixing agent for said dye, and creping the sheet so treated.

4. A method of making non-bleeding crepe paper, comprising the steps of treating a sheet of tissue paper with a creping bath characterized by containing a dye, glue, and a fixing agent for said dye, and creping the thus treated sheet. 70

5. A method of making non-bleeding crepe paper, comprising the steps of treating a sheet of tissue paper with a creping bath characterized by containing a basic dye, hide glue and a fixing agent for said dye, and creping the thus treated sheet. 75

6. A method of making non-bleeding crepe paper, comprising the steps of treating a sheet of tissue paper with a creping bath characterized by containing a basic dye, glue, and a direct dye and creping the thus treated sheet. 80

7. A method of making non-bleeding crepe paper, comprising the steps of treating a sheet of tissue paper with a creping bath characterized by containing a dye, glue, and a direct dye as a fixing agent or mordant for said first dye, and thereafter creping the sheet. 85

8. A creping bath, characterized by containing a dye, a protective colloid, and a fixing or mordanting agent for said dye. 90

9. A creping bath, characterized by containing a dye, an adhesive protective colloid, and a fixing agent or mordanting agent for said dye. 95

10. A creping bath, characterized by containing a dye, an adhesive protective colloid, and a direct dye, as a fixing agent or mordant for the first dye. 100

11. A creping bath, characterized by containing a dye, glue and a fixing agent for said dye. 105

12. A creping bath, characterized by containing a basic dye, glue, and a fixing agent for said dye. 110

13. A creping bath, characterized by containing a basic dye, glue and a direct dye serving as a fixing agent or mordant for said first dye. 115

Signed by us at Framingham, Massachusetts, this eleventh day of June, 1929. 115

GARDNER R. ALDEN.  
THOMAS NELSON.

120

125

130